

# United States Patent Office

2,920,362

Patented Jan. 12, 1960

1

2,920,362

## METHOD OF REFINING METAL

Davidlee Von Ludwig, Brooklyn, N.Y., assignor to Selas Corporation of America, Philadelphia, Pa., a corporation of Pennsylvania

No Drawing. Application May 22, 1953  
Serial No. 356,871

1 Claim. (Cl. 22—216)

The present invention relates to the refining and densifying of metals, and more particularly to the use of vibration during the refining period. The present application is a continuation in part of my copending application, Serial No. 61,132, filed November 19, 1948, now abandoned.

Prior efforts to refine metals in vacuum have not been commercially successful for several reasons. The time required to obtain an appreciable freedom from gaseous impurities in the metal when the cycle of outgassing normally attempted in vacuo has been used has been excessive, and the degree of purification obtainable in such treatments has not been as great as desired. The best prior technique employed for vacuum refining metals has been incapable of reducing the quantity of non-gaseous impurities, such as slags, stable oxides or nitrides or other metalloids contained in the melt. These deficiencies have been the basis for beliefs that no benefits of practical value can accrue from the production of castings in vacuum. While it is desirable to remove non-metallic contaminants from ingots to be subsequently remelted and formed into castings, it is even more important to produce ingots free from discrete solid impurities when such ingots are to be forged or otherwise mechanically worked. In such cases minute impurities that might not produce a fault in a cast structure, when elongated by forging or other working, frequently become sources of weakness on preferred lines of metal breakdown. In most cases fatigue failure planes are of far greater proportional magnitude to the reliability of forged structures than to cast structures.

It is an object of the present invention to provide a method of removing gases and slags or other undesirable stable contaminants from metal. It is a further object to provide a method of refining or purifying metals or alloys more rapidly and to a higher degree than has hitherto been possible.

In following my invention the metal to be refined may be melted in a high vacuum. While in its molten state the metal is subjected to vibration of controlled frequency and amplitude so that the melt is thoroughly agitated. Such vibrations produce a segregation of the metal and the contaminants in accordance with their relative specific gravities. The vibration also speeds up appreciably the precipitation and expulsion of any gas that may be in the metal, and materially increases the effectiveness of gas removal.

It is a further object of my invention to use controlled vibrations to precipitate and segregate undesired constituents from a body of metal being refined and purified during the period of solidification of the metal in the ingot molds.

It is a further object of my invention to use controlled vibrations to produce cast ingots intended for use as forging stock or other mechanical reforming base metal, wherein by means of the correct frequencies and amplitudes of vibration, not only are gaseous and solid contaminants removed from the metal, but the grain size is

2

controlled and the segregation of alloying elements in the ingot mass controlled.

The various features of novelty which characterize my invention are pointed out in the claim annexed to and forming a part of this specification. For a better understanding of the invention, however, its advantages, and specific objects attained with its use, reference should be had to the description set forth in detail below.

In accordance with the principle of this invention, if 5 the treatment is to take place in an environment of sub-atmospheric pressure, relatively large masses of metal, either pure or of some particular alloy, are placed in a melting crucible and the crucible put in an apparatus and tightly sealed. The pressure in the apparatus is then 10 decreased until a suitable value thereon has been reached. This value is effectively between one and ten microns mercury pressure, except when the melt contains metals which sublime, boil, or otherwise are lost from the melt at such pressures. In this case the degree of evacuation used 15 in the refining chamber will be as low as possible but high enough to avoid excessive metal loss. During the time that the pressure change is taking place, or after the proper pressure level has been attained, the crucible and charge will be heated to melt the metal by electric resistance or induction coils or by suitably muffled gas or oil 20 burners. The temperature of the melt will be maintained sufficiently above the melting point to insure complete liquidity in order to permit ready escape of gases, a uniform temperature being held until pressure equilibrium 25 is attained. In this invention the molten metal is to be subjected to vibration from the moment liquefaction is complete in order to expedite the expulsion of gases, throughout the period of holding at constant temperature while 30 stabilizing the system pressure. While the melt is being vibrated, after the pressure has been stabilized at the highest temperature to which the metal is subjected, the heat input is stopped and the melt is cooled until solidification has commenced, while the vibration is continued. 35 Cooling is expedited by passage of water through the induction coils, or by passages provided in the apparatus for that purpose. The metal is then remelted preparatory to discharge from the crucible into ingot molds of suitable sizes and shapes. If desired, the metal can be 40 poured without freezing and remelting. While the metal is being poured into the ingot molds, the molds are caused to vibrate, preferably in a vertical plane, for the purpose of separating the stable non-gaseous slags or other impurities which could not be removed in the prior 45 phases of the refining treatment. After solidification of the ingots is complete, the pressure in the apparatus may be returned to atmospheric. It is generally desirable to transfer the hot, refined ingots to a cooling chamber in which a suitable controlled atmosphere can be maintained in contact with the cooling metal to minimize the 50 depth of oxide or nitride or other contamination of the ingot surface. Almost total exclusion of gas and solid contaminants can be obtained during the refining cycle mentioned above if the metal is vibrated at the correct frequency and in the proper direction during the cooling and slow solidification phase of the refining cycle. The vibration can and should also take place during the cooling of the metal in the ingot molds until the ingots are completely frozen. 55 In casting ingots of refined and degassed metal for subsequent remelting and casting into desired shapes, the chief characteristic required is that of the exclusion of slags or other non-metallic stable contaminants. If no particular effort is made to avoid segregation or erratic grain growth, the vibration frequency and amplitude can be the same for most alloys. The grain growth and alloy segregation are automatically corrected when the in- 60 65 70

gots are remelted for casting to the desired shapes. The term vibration as used herein should not be confused with ordinary shaking or stirring of the metal.

The vibration producing effective exclusion of gases, slags and stable metalloids from metals and alloys will vary with the composition of the material being treated. It is necessary to determine the proper frequency range of the vibrations as well as the range of amplitude and planes of orientation. My experiments indicate that each group of alloys based upon any particular metal or metal group has a sufficiently broad range of response to permit of practical controls being established for alloy groups rather than for each individual alloy. The above noted range of the vibrations for any particular metal or family of alloys must be determined empirically. The proper amplitudes and frequencies which produce improved cleanliness of metals when applied to them in a vacuum are the same as those determined upon the metal in normal air pressures. Therefore, the experimental determination of the proper vibrations for any given composition may be determined without difficulty outside the vacuum environment. Generally these vibrations that speed up degassing and produce segregation of impurities will have frequencies in the range of from 500 to 5000 cycles per minute with an amplitude within the range of from  $\frac{1}{64}$ " to  $\frac{1}{32}$ ". The vibration preferably is directed in a vertical plane and has the form of a sine wave. The ingots so produced will be found to have most of the impurities in the top or bottom layer of metal, depending upon the relative specific gravities of the impurities and the metal containing them. Once isolated in these specific ingot sections, it becomes a simple matter to grind or machine away the layers containing the impurities.

The proper vibrations to be applied during the several phases of the refining cycle are determined in accordance with the function they are intended to perform. Most effective exclusion of gases is obtained by vibration during the period of cooling and slow, controlled solidification in the crucible during which the entire melt is vibrated prior to being reheated for casting into ingots. For the purpose of segregating non-gaseous contaminants, the ingot molds are vibrated during the time of solidification of the ingot metal, the vibration to have commenced as soon as the metal begins to fill the ingot molds. The vibration may be accomplished by a stirring mechanism which is equipped with a vibrating device the stirring mechanism would then impart the vibrations to the molten metal. In some cases, for the reasons of chemistry or temperature or both, no suitable material for the stirring device may be available. The metal may then be caused to vibrate by means of a device fastened to the crucible or the ingot molds or the supports therefore. Preferably the vibrating device, of what ever kind used, will be self contained and electrically operated, so that no moving connections are required to extend through the walls of a vacuum tight container when the refining is taking place in such a container.

When the metal being refined is to be used for forging or to be otherwise cold or hot worked without being reliquified, the vibration treatment must be accurately regulated while the metal is being cast into the ingot molds and while it is solidifying therein. Whereas the low frequency vibration of the ingot molds in the vertical plane will in all cases separate the non-gaseous contaminants, it will also tend to cause the various alloying elements not in true solution in the base metal to be undesirably separated. Both alloy segregation and grain size may be controlled by the use of a high frequency vibration of low amplitude applied in any convenient direction and of such an order of magnitude, with respect to the low frequency vibration being simultaneously applied, as to avoid the establishment of nodes of interference or amplification of the several wave patterns. Such vibration may be imparted to the ingot mold by any

well known high frequency vibrating device in which the vibrations produced can be controlled as to frequency and amplitude. My work has demonstrated that it is possible to attain a controlled grain size of almost any desired magnitude by the correct use of the high frequency, low amplitude vibration in conjunction with the low frequency vibration and that, all other factors being equal, the grain size in the solidified ingot becomes increasingly smaller as the frequency of vibration rises.

When a high frequency, low amplitude vibration is used, the values thereof must be determined empirically in the manner described above. This vibration will generally be from 2500 cycles per minute to 35000 cycles per minute, but will in all cases be at least ten times as fast as the low frequency vibration and never an exact multiple thereof. The amplitude will be in the range of from 0.0005" to 0.005" though generally speaking 0.001" has been adequate and no apparent gain is attained by an excessive amplitude of vibration at the higher frequency.

20 The wave form of the low frequency vibration will take the form of a sine curve when producing ingots which are to be forged, in order to avoid inter-granular cracking and other mechanical weakening of the ingot structure. Whether one or two vibrations are used, the ingot should be vibrated during solidification until all metal phases are solid. The entire ingot mass solidifies at a higher temperature level than normally is attained in the solidification of metal without the use of vibration. This fact further reduces the time of the vacuum refining treatment.

25 While the use of vibration in refining and degassing metal is advantageous in any environment, it is particularly advantageous when used in a refining operation taking place in vacuum.

30 As a specific example of a treatment of one alloy and the improved results that are obtained, the following is given.

35 In this example, the metal treated is an alloy of aluminum consisting of 5% silicon and 95% aluminum. The alloy is placed in a crucible which is surrounded by a 40 container that is evacuated. Evacuation and heating of the alloy are started and the rate of evacuation is such that a pressure which is equivalent to one micron of mercury is obtained by the time the alloy has reached a pasty condition indicating that it is at a point of transition from a solid to a liquid. The pressure of the 45 container in which the melting takes place is at about one micron of mercury or at a partial pressure that is equivalent thereto, which can be about 50 microns of mercury with an atmosphere neutral to the metal such as helium or argon. The purge pressure of about 50 microns of inert gas is physically and chemically the same as a total vacuum in as far as the equilibrium of dissolved gases in the metal is concerned and can be obtained in considerably less time and with less equipment 50 than is required for a higher vacuum. During the time that the metal is melted, and beginning at the time that it starts to change from solid to liquid, vibration is applied to the crucible in which the melting is taking place. This vibration is in any direction at a frequency of 5,000 55 cycles per minute and an amplitude of 0.05". The vibration, along with the reduced atmosphere causes the dissolved gases in the alloy to be expelled or precipitated.

60 After the metal is liquefied, it is held at its liquid temperature of between 1225° F. to 1300° F. while being vibrated until such time as the pressure in the container reaches equilibrium, indicating that the dissolved gas in the metal has been removed for the temperature equilibrium of the liquid metal. The metal is then solidified by cooling it in any desired manner, and the vibration 65 must be maintained until the melt has solidified. The entire time for degassing will take from 30 to 45 minutes as compared to over 10 hours at the same pressure if no vibration is used. The reduced atmospheric pressure around the crucible should be maintained, however.

70 The metal is then remelted and discharged into in-

got molds. For this purpose, it is desirable to use a bottom discharge type of crucible, since the casting can be easier accomplished in a container having a reduced atmosphere with such a crucible than if some mechanism is required to tilt the crucible for pouring. If the ingots are to be remelted, the form of the grain structure produced is more or less immaterial since any grain structure that is obtained would be lost upon remelting for casting. During the casting, however, the ingot mold is vibrated at a frequency of about 2500 cycles per minute and the amplitude ranging from  $\frac{1}{16}$  to  $\frac{3}{32}$  of an inch. These vibrations are applied in a vertical direction and have the form of an undamped sine wave. The purpose of this vibration and its practical effect is to separate various insoluble contaminants and slag which will segregate to either the top or the bottom of the ingot depending upon the relative specific gravity of the alloy and the contaminants. In this aluminum alloy, the drosses are forced to the top. Upon solidification and cooling of the ingots, the contaminants can then be removed by grinding or machining them from the end of the ingot.

If the ingots are to be used directly for forging or rolling or other purposes, the vibration of 2500 cycles per minute with an amplitude of  $\frac{1}{16}$  to  $\frac{3}{32}$  of an inch is applied as in the above example. There is also applied a second vibration of a frequency of approximately 26000 cycles per minute, or at least ten times the low frequency vibration, and an amplitude of 0.005". This vibration is also an undamped sine wave but it can be applied in any direction as long as it is applied to the mold and has an effect upon the molten metal. The low frequency, high amplitude vibration in this case also serves to segregate the impurities from the metal of the alloy. The high frequency and low amplitude vibration serves to prevent segregation of the alloy constituents and to produce a fine, dense grain in the alloy, eliminating center shrinkage or pipe.

In either case, whether the ingot is to be remelted or is to be used for rolling or forging the vibrations are continued until solidification of the metal is completed.

The above treatment will produce metal with a tensile strength in the neighborhood of 27,000 pounds per square inch with an elongation of from 10% to 30% coupled with extremely fine, dense grain structure. This particular alloy with ordinary casting will have a tensile strength of about 17,000 pounds per square inch with from 3% to 6% elongation. It will, therefore, be seen that the physical qualities of the alloy are greatly improved by the application of the vibration during the refining process.

The method of treating metal described above is equally as effective on other metals such as copper and ferrous alloys, for example, when the frequencies and amplitudes of the vibrations have been determined in the manner described above.

The above specific example of the treatment of a given aluminum alloy was described as taking place in a reduced atmosphere. The same treatment can, of course, take place in the air at atmospheric pressure. In such a case, however, there is some loss of maximum outgassing. Maximum segregation of impurities and refinement of

the metal grain structure can be obtained by the use of the high frequency, low amplitude and low frequency, high amplitude vibrations regardless of the environment in which they are applied.

5 The application of vibrations to metal during refining not only decreases the time required for treatment at any given temperature pressure level to produce thorough outgassing of the metal, but also, when used in the manner outlined above, effectively segregates the non-gaseous 10 contaminants such as slags, stable oxides, nitrides, sulfides and similar metalloids, concentrating these undesirable elements in specific layers of the ingot metal, either at the top or bottom of the metal mass. Use of 15 vibrations in the manners outlined above not only accelerates the tendency for gases to separate themselves from the metal, but also overcomes the tendency for the precipitated gases to be held as discrete voids within the solidifying metal, wherefrom they may be readily re-dissolved upon subsequent remelting of the ingot, or where- 20 in they may become the source of mechanical flaws in the body of the object which has been formed from the ingot metal containing trapped gas bubbles.

While in accordance with the provisions of the statutes, I have described the best embodiment of my invention now known to me, it will be apparent to those skilled 25 in the art that changes may be made without departing from the spirit and scope of the invention as set forth in the appended claim, and that in some cases certain features of the invention may be used to advantage without a corresponding use of other features.

What is claimed is:

The method of processing metal to remove gas and non-metallic contaminants which comprises placing the metal in an enclosed space, reducing the pressure in said 35 space to an effective pressure below 50 microns of mercury, applying heat to the metal to melt the same and reaching the minimum pressure by the time the metal has been heated to a temperature at which it is beginning to liquefy, vibrating the metal at a frequency of from 40 500 to 5000 cycles per minute at an amplitude of from  $\frac{1}{64}$ " to  $\frac{3}{32}$ " from the time it begins to liquefy, after the pressure in the space has reached equilibrium pouring the metal into a mold, vibrating the mold in a vertical direction at a frequency of from 500 to 5000 cycles 45 per minute at an amplitude of from  $\frac{1}{64}$ " to  $\frac{3}{32}$ " from the time pouring is started until solidification in the mold is complete, and returning the pressure in the space to atmospheric.

References Cited in the file of this patent

UNITED STATES PATENTS

|           |            |               |
|-----------|------------|---------------|
| 1,318,740 | Fessenden  | Oct. 14, 1919 |
| 1,956,910 | Roth       | May 1, 1934   |
| 2,660,414 | Von Ludwig | Nov. 24, 1953 |

FOREIGN PATENTS

|         |               |               |
|---------|---------------|---------------|
| 138,648 | Great Britain | May 5, 1921   |
| 683,996 | France        | Mar. 10, 1930 |
| 456,657 | Great Britain | Nov. 9, 1936  |
| 479,933 | Great Britain | Feb. 8, 1938  |
| 480,554 | Great Britain | Feb. 24, 1938 |